

Sept. 10, 1935.

G. E. SIEVERT

2,014,148

PREPARATION OF LEAD BORATE

Filed July 18, 1933



BY

GUILIO E. SIEVERT *INVENTOR*  
*James M. Abbott* ATTORNEY

## UNITED STATES PATENT OFFICE

2,014,148

## PREPARATION OF LEAD BORATE

Guilio E. Sievert, South Gate, Calif.

Application July 18, 1933, Serial No. 680,987

2 Claims. (Cl. 204—9)

This invention relates to the preparation of lead borate and its use in glazes for ceramic coatings.

In the glazing of pottery it is necessary to apply a glazing material to the surface of the article of pottery and to thereafter heat the article until a suitable glaze has been produced.

In common practice certain ingredients of glazing material are usually formed in what is known to the trade as a frit which is fired and must then be ground to a desired degree of fineness before it is applied to the article. In practice it is found that in some instances subsequent firing of the pottery causes cracks to form in the glaze material which sometimes results in causing the glaze to peel away from the body before fusion occurs.

It is the principal object of the present invention to provide a product, a process of its production, and use upon articles of pottery, which product may be directly prepared without being formed as a frit and then ground; may be easily applied, and will at suitable temperatures produce a desirable uniform glaze.

The present invention contemplates the production of lead borate as a glazing substance and means for using this product.

The invention is illustrated by way of example in the accompanying drawing in which:—

The figure is a view in diagram showing the flow plan of the process with which the present invention is concerned.

Referring more particularly to the drawing, 10 indicates an electrolytic precipitation cell having cathode plates 11 therein, and one or more anode plates 12. Diaphragms 13 and 14 are interposed between the cathode and anode plates and are of such a character as to permit ionization currents to flow while retarding the mingling of the electrolyte solution from the area occupied by the anode with the solution in the area occupied by the cathode. The anode is formed of lead. The cathodes are preferably formed of steel or other metal which will not react to the materials in solution. A case 15 is provided for the precipitation cell 10, and is here shown as formed with two draw off pipes 17 and 18 through which electrolyte solution may be drawn through a pipe 19 to a catholyte tank 20. The liquid within this tank may be returned to the cathode portion of the cell 15 through a pipe 21 and by suitable means such as pump 22. The catholyte solution has a boric acid content. The solution has been made by

dissolving boric acid in relatively small quantities of hot water before being added to the solution of sodium acetate or an equivalent chemical element. It is preferable that the strength of the solution shall be of the order of a saturated boric acid solution at 25° C. The boric acid thus formed is added to a solution of sodium acetate. Such a solution, containing two ounces of sodium acetate to a gallon has been found to be suitable. The boric acid is introduced into the sodium acetate solution while hot and until a saturated solution of boric acid is made. 5

It is desirable to maintain such a solution in the catholyte section of tank 20. This may be done by replenishing the boric acid solution with 15 the sodium acetate solution of the strength previously described.

The anolyte solution occurring in the portion of the precipitation cell occupied by the anode 12 is drawn from the bottom of the container 15 20 at 23, and is led through a pipe 24 to a lead borate settling tank 25. The lead borate will settle out of the solution and may be drawn from the bottom of the tank 25 through a pipe 26. The anolyte accumulating above the lead borate in the tank 25 is drawn from the top of the tank through a pipe 27 and is conveyed to an anolyte storage tank 28. This anolyte is returned to the portion of the cell 10 occurring 30 between the diaphragms 13 and 14 through a pipe 28'. This may be accomplished by a pump 29.

The lead borate which is drawn through the pipe 26 is delivered to suitable washing and filtering equipment generally indicated at 30. The liquid from this equipment is delivered into the anolyte tank 28 while the filter cage is drawn from the filtering equipment, dried and then placed in containers. The final product will be a 40 high grade of lead borate which may then be used as a glazing material in pottery work. 35

The electrolytic cell 10 which is used may employ any desired direct current, but in practice it has been found that a current having voltage 45 of from 3½ to 6 volts, and an amperage in the order of 15 amperes per square foot of anode surface, nearness of the anodes to the cathodes, strength of solution and temperatures to obtain a satisfactory maximum precipitate of lead. 50

After the lead borate has been filtered and dried it is then ready for use in a glaze formula designed for a particular purpose. A typical glaze formula for producing sanitary ware with a white glaze is set forth in percentages of raw materials 55

instead of frit, which would be normal procedure, as follows:

|                     | Per cent |
|---------------------|----------|
| Silica              | 24.79    |
| 5 Lead borate       | 19.32    |
| Ball clay           | 0.62     |
| Calcined china clay | 4.05     |
| Raw china clay      | 1.41     |
| Feldspar            | 21.25    |
| 10 Whiting          | 3.48     |
| Zinc oxide          | 7.37     |
| White lead          | 9.21     |
| Tin oxide           | 8.50     |

- 15 In preparing sanitary ware with lead borate it is fired in the usual manner, but upon observation it is found that the action of the glaze during the firing operation and the resultant product obtained is much more desirable than that obtained 20 by the use of the well known boric acid method now in use, and which requires the preliminary making of a frit. The glaze material is more uniform in consistency and is easier to handle and to apply to the ware. It also has been demonstrated 25 by its use that it will fuse at a much lower temperature than most other glaze materials, and that in addition the fusion takes place without an initial cracking or blistering of the glazed material, but with an even uniform fusion. The 30 character of the lead borate is such as to insure that it will melt before any such objectionable cracking occurs, and that it will be withdrawn from the fire in more satisfactory condition and with less possibility that the product will be rejected.

In the production of the lead borate it will be evident from the examination of the flow plan that the electrolyte may be maintained in continuous circulation so that ingredients which 40 precipitate out due to the electrolytic and chemical reactions within the precipitation cell 10 may be replenished constantly, and so that the lead borate precipitate may be constantly drawn away and prepared for use.

45 It is to be understood that while the cell 10 is shown with only one anode and two cathodes, any number of each might be used. However, it is

preferable to provide one more cathode than anode.

It will, of course, be understood that this material might be made by drawing off the entire quantity of electrolyte continuously and passing 5 it through the settling tank 25, after which a replenished electrolyte solution would be returned to the precipitation cell 10 and would be used to submerge the cathodes and the electrodes.

It will thus be seen that the invention here disclosed provides simple apparatus and a simple method for producing a glazing product, and for insuring that said product may be made uniformly and economically, and that the glazed ware obtained as a result of its use will be of high 15 quality.

While I have shown the preferred form of my invention, the method of making the same, and of using the product, it will be understood that various changes might be made in the method, 20 apparatus and proportions of parts by those skilled in the art without departing from the spirit of the invention as claimed.

Having thus described my invention, what I claim and desire to secure by Letters Patent is:— 25

1. A method of producing lead borate within an electrolytic cell characterized by having a lead anode and metallic cathodes separated from each other by diaphragms through which electric current may flow, thereafter continuously introducing a boric acid containing electrolyte into the space occupied by the cathodes and continuously withdrawing the electrolyte from the space occupied by the anode, said withdrawn electrolyte containing lead borate. 30

2. A method of producing lead borate within an electrolytic cell characterized by having a lead anode and metallic cathodes separated from each other by diaphragms through which electric current may flow, thereafter continuously introducing a boric acid containing electrolyte into the space occupied by the cathodes and continuously withdrawing the electrolyte from the space occupied by the anode, said withdrawn electrolyte containing lead borate, and then separating the 40 lead borate precipitate from the solution. 45

GUILIO E. SIEVERT.